

Patented May 3, 1927.

1,627,254

# UNITED STATES PATENT OFFICE.

BURGESS W. SMITH, OF ROCHESTER, NEW YORK, ASSIGNEE TO THE TODD COMPANY, INCORPORATED, OF ROCHESTER, NEW YORK, A CORPORATION OF NEW YORK.

## SAFETY PAPER.

No Drawing.

Application filed August 13, 1925. Serial No. 50,136.

This invention relates to safety or fraud preventative paper for use, for example, for making checks, drafts, bonds and other paper instruments, and more particularly 5 to the variety of such paper having a chemical ingredient incorporated therein for reaction with ink eradicating substances in such a manner as to indicate and warn of attempted alterations, the chief object of 10 the invention being to provide an efficient paper of this nature adapted to be economically manufactured in a wide variety of styles and colors, and to be quickly and sharply changed or deepened in color by 15 the application of an ink eradicator to afford a conspicuous, substantially permanent warning of attempts to alter matter written thereon.

To these and other ends the invention 20 resides in certain improvements and combinations of parts, all of which will be hereinafter more fully described, the novel features being pointed out in the claims at the end of the specification.

25 Safety papers have been made with chemical substances incorporated in them for reaction with ink eradicators to indicate attempts at alteration by the development of a change in color. Such papers, however, 30 have generally been open to the objection that the chemicals employed have in one way or another been unsatisfactory, either because insufficiently sensitive in reaction with eradicators, or because the products of 35 such reaction have been relatively soluble or reducible to colorless compounds and capable of removal from the paper, or for other reasons. It has been found that these difficulties are overcome with marked success through the incorporation in the paper 40 of certain organic substances found to possess the various qualifications essential to the production of a commercially practical and efficient safety paper. These substances 45 belong to a related group or family characterized by the presence of naphthalene or anthracene rings, and their essential characteristics are believed to be due to the presence 50 of a molecular configuration or arrangement comprising a naphthalene or anthracene radical or analogous group of rings having a carbon atom directly joined to a carbon atom of another carbon ring or group of rings and having a plurality of amino radicals substituted for hydrogen atoms. Among 55

the substances of this class, for example, are those characterized by the presence of two naphthyl radicals joined together in such a manner that an alpha carbon atom of one is joined directly to an alpha carbon atom of 60 the other and in which the amino radicals occupy any of the various positions in this formation and preferably the para position to the linkage, which latter is the characteristic of the best known substance in this 65 class, i. e., alpha-naphthidine. The structure of the latter is illustrated in graphic form as follows:



This is a solid reacting with oxidizing 75 agents, such as sodium hypochlorite, to yield crimson or purplish precipitates of a high degree of color value and insolubility. The various isomers of this compound, such as dinaphthylene, have the same characteristics, but as far as investigated have not the desired characteristics to the same extent. For example, their salts are relatively 80 soluble, while the basic substances have the same characteristics described above. 85

It is believed that this configuration need not be symmetrical, but that the groups may vary in the number of carbon rings and in the disposition of the amino radicals. For example, the compound may be composed of 90 a radical or group known as the anthracene ring coupled to the group known as a naphthalene ring, and the disposition of the amino radicals may be in various positions thereof. 95

It is preferred to use the salts as, for example, the sulphates or chlorides, as they have greater stability than the base under the influence of moisture and light rays and because the reaction precipitates are more 100 firmly held to the paper. The sulphates have been found suitable for the purposes of this invention. It is probable however that there are other compounds having the essential characteristics described above, as 105 well as their salts, which may be used with substantially the same success.

The above substances are affected little when subjected to atmospheric conditions or strong light for an indefinite period and, in 110

addition to this advantageous feature, they are highly sensitive to the usual ink eradicating chemicals such as potassium dichromate, potassium permanganate, hypochlorite, and other oxidizing substances in reaction with which they afford precipitates which are conspicuously deep in color as well as relatively insoluble and from which the color is not discharged by the usual reducing agents. When an eradicating chemical is applied to safety paper containing one of these substances, the latter reacts quickly and sharply to develop a conspicuous color over the area treated and the relatively insoluble stain thus produced affords a conspicuous warning of an attempt at erasure. A further advantage of the substances described lies in the fact that they are practically colorless and may therefore be employed to produce white safety paper, or may be readily employed with paper having a desired tint or color, while of course any known and suitable coloring matter may be added to these compounds as may be desired.

In the incorporation of a sensitive compound of the class described the quantity to be employed varies of course with the depth of stain desired upon reaction, the rate of absorption by the paper, the apparatus used and other factors understood in the art. It has been found that for a ton of pulp when added in the beater or jordan, thirty pounds is sufficient of a substance of the above character which I believe to be alpha-naphthidine sulphate and which I prepare by the oxidation of alpha-naphthylamine in sulphuric acid with ferric oxide, as described by F. Reverdin and C. De La Harpe in the Chem. Ziet. 16, 1687. The resultant of this reaction is believed to be alpha-naphthidine sulphate, somewhat contaminated with the various isomers and incidental byproducts; nevertheless the material prepared as described is well suited for the purpose outlined without completely isolating the base where it is desired to use the sulphate.

The chemical ingredients described may be added to the paper after the latter is formed by passing the web through baths or by incorporating it in the sizing itself. Furthermore, the low relative solubility of some of the salts admits of their production in the web itself by double decomposition. For example, such insoluble salts may readily be formed by impregnation of the paper with a soluble salt of the base, and then by passing the web through an acid or salt of an acid such as sulphuric acid or sulphate of soda, which will by double decomposition produce the desired insoluble salt, or the base may be dissolved and the salt formed by acids in the same manner. A chemical ingredient of the class described thus has an additional advantage of being

suitable for incorporation in the paper economically in accordance with known and practical methods.

I claim as my invention:

1. A safety paper having incorporated therewith an organic compound having a molecular arrangement comprising a group of carbon rings joined together by having two carbon atoms in each ring in common with the adjacent ring, a carbon atom of said group of rings being attached to a carbon atom of another carbon ring, and a plurality of amino radicals substituted in said rings for hydrogen atoms, said compound being deepened in color by reaction with ink eradicating chemicals. 70 75

2. A safety paper having incorporated therewith an organic compound having a molecular arrangement comprising a group of carbon rings joined together by having two carbon atoms in each ring in common with the adjacent ring, a carbon atom of said group of rings being attached to a carbon atom of another group of carbon rings similarly bound together and a plurality of 80 85 90 amino radicals substituted in said rings for hydrogen atoms, said compound being deepened in color by reaction with ink eradicating chemicals.

3. A safety paper having incorporated therewith a salt of a basic organic compound having a molecular arrangement comprising a group of carbon rings joined together by having two carbon atoms in each ring in common with the adjacent ring, 100 105 a carbon atom of said group of rings being attached to a carbon atom of another carbon ring, and a plurality of amino radicals substituted in said rings for hydrogen atoms, said compound being deepened in color by reaction with ink eradicating chemicals.

4. A safety paper having incorporated therewith a salt of a basic organic compound having a molecular arrangement comprising a group of carbon rings joined together by having two carbon atoms in each ring in common with the adjacent ring, a carbon atom of said group of rings being attached to a carbon atom of another group of carbon rings similarly bound together 110 115 and a plurality of amino radicals substituted in said rings for hydrogen atoms, said compound being deepened in color by reaction with ink eradicating chemicals.

5. A safety paper having incorporated therewith an organic compound having a molecular arrangement comprising a group of carbon rings joined together by having two carbon atoms in one ring of the group in common with an adjacent ring, a carbon 120 125 atom of said group of rings other than one of said common carbon atoms being linked to a carbon atom of another carbon ring, and a plurality of amino radicals substituted in said rings for hydrogen atoms, said 130

compound being deepened in color by reaction with ink eradicating chemicals.

6. A safety paper having incorporated therewith a compound of the aromatic series having carbon rings with two carbon atoms in common and also having carbon rings with carbon atoms linked together, and a plurality of amino radicals substituted in said rings for hydrogen atoms, said compound being deepened in color by reaction with ink eradicating chemicals.

7. A safety paper having incorporated therewith an organic compound having a plurality of carbon rings comprising two types of ring connections, one being by means of two carbon atoms in common, the other being the chain type of connection, and a plurality of amino radicals substituted in said rings for hydrogen atoms, said compound being deepened in color by reaction with ink eradicating chemicals.

8. A safety paper having incorporated therewith an organic compound having a molecular arrangement characteristic of alpha-naphthidine and its salts. 25

9. A safety paper having incorporated therewith a sulphate of an organic compound whose molecular arrangement comprises a group of carbon rings joined together by having two carbon atoms in each 30 ring in common with the adjacent ring, a carbon atom of said group of rings being attached to a carbon atom of another carbon ring and a plurality of amino radicals substituted in said rings for two hydrogen atoms, said paper being deepened in color by reaction with chemical ink eradicators. 35

10. A safety paper having alpha-naphthidine incorporated in the body or sizing thereof.

BURGESS W. SMITH.